

## UNITED STATES PATENT OFFICE

2,241,742

PROCESS OF PRODUCING ALKALINE-EARTH  
MOLYBDATES IN LUMPS

Gustav Schliphaus, Hamburg-Harburg, Germany

No Drawing. Application December, 15, 1938,  
Serial No. 245,983. In Germany July 14, 1938

12 Claims. (Cl. 75—133)

This invention relates to a process of producing alkaline-earth molybdates in lumps.

In the production of molybdeniferous special irons and steels ferromolybdenum is increasingly replaced by combinations of molybdcic acid with other metals, preferably metals of the alkaline-earth group like calcium. The molybdenum content of these molybdenum compounds is reduced by the liquid iron to metallic molybdenum which is absorbed by the iron.

The use of these compounds affords considerable advantages compared with that of ferromolybdenum, since they can be produced in a substantially purer form, particularly without carbon content, and the cost of production is much lower than that of ferromolybdenum. The present state of the art with respect to producing compounds of molybdcic acid and alkaline-earth metals is, however, open to the objection that they are obtainable only in pulverulent form and not in that of solid lumps of larger size.

When a hot iron or steel bath is charged with this fine powder, much dust develops and involves a considerable loss of expensive molybdenum compounds, in consequence whereof most of the economic advantages realized by the replacement of ferro alloys are lost again.

It has been proposed to moisten a mixture of molybdcic acid and calcium carbonate, to press the paste, to dry the pieces thus obtained and to feed them to the iron or steel bath. Subjected to the heat of the furnace, this mixture will form calcium molybdate. However, as molybdcic acid becomes volatile if exposed to heat, a portion thereof will be lost. Furthermore, since the firm structure of the pieces or lumps is eliminated due to the escape of the carbonic acid, they will crumble, so that the result is substantially the same as if pulverulent calcium molybdate had been added at first.

Compared with the known art, the invention consists in employing as addition to the iron or steel bath finished lumpy compounds of molybdcic acid and alkaline-earth metals, which do not volatilize when subjected to heat and which do not crumble when heated.

It has been found that such compounds of molybdenum and alkaline-earth metals can be produced in the form of lumps or pressed pieces in the manner described below. Their use affords the great advantage that the production of the molybdcic acid compounds as well as their addition to an iron or steel bath are effected without any loss of valuable metal.

From the raw material containing molybdenum, molybdcic acid is obtained in known manner whose content of constituents detrimental to iron or steel is within permissible limits. The molybdcic acid is thoroughly mixed with the hydroxide of an alkaline-earth metal, as calcium hydroxide, in the stoichiometric ratio corresponding to the normal or an acid molybdate (polymolybdate), with a slight addition of water if necessary, and pressed in suitable molds by the application of great pressure. The pressed pieces thus obtained are hardened by drying, and there occurs an extensive combination of molybdcic acid and alkaline-earth hydroxide while neutral or acid molybdate (polymolybdate) is formed.

To provide for the complete chemical conversion of the molybdcic acid and alkaline-earth hydroxide and to insure greater hardness and strength of the pressed pieces it is advisable to soak the latter with water. This can be done by placing them for some time in a vessel filled with water and thereupon drying them in a suitable apparatus while subjecting them to heat so as to cause evaporation of the water, or by treating them in a hardening boiler with steam under pressure, or by exposing them in a suitable vessel to the action of a current of superheated steam.

From the mechanical mixture of the two substances a chemical compound is thus produced which retains the original outer shape of the pressed piece and possesses extraordinary mechanical strength. The hardened pressed piece does not crumble even when exposed to the high temperatures of an iron or steel bath, so that loss due to dusting is excluded.

The peculiar advantage afforded by the process according to the invention is that the lumpy shape is not brought about by means of an additional binding agent but by converting the mechanical mixture of two substances into a chemical compound.

In the same way neutral and acid molybdates (polymolybdates), such as

$\text{CaO} \cdot \text{MoO}_3$ ,  $\text{CaO} \cdot 3\text{MoO}_3$ ,  $\text{CaO} \cdot 4\text{MoO}_3$ ,  
 $\text{CaO} \cdot 8\text{MoO}_3$ ,  $\text{CaO} \cdot 12\text{MoO}_3$

may be obtained, depending on the mixing proportion of molybdcic acid and calcium hydroxide or of the hydroxide of another alkaline-earth metal, for instance of barium or strontium.

The pressed pieces are preferably produced so as to have equal molybdenum contents to facilitate their subsequent use.

These pressed pieces consisting of neutral or acid molybdates (polymolybdates) of alkaline-earth metals may be produced also in the same manner but with an addition of silicic acid, as quartz sand, by uniformly distributing the sand in the mixture formed of molybdic acid and alkaline-earth hydroxide prior to molding and pressing. Owing to the presence of silicic acid in the pressed piece consisting for instance of calcium molybdate the formation of calcium silicate becomes possible after the melting and reduction of the molybdic acid, which with respect to its lime and silica content corresponds to steel furnace slag.

The following examples show the performance of the invention:

*Example 1*

For the production of normal calcium molybdate  $\text{CaO}_3\text{MoO}_3$ , 90 g. of commercial molybdic acid containing 64.4% Mo=57.96 g. Mo are mixed with 45.6 g. of commercial 98 per cent. calcium hydroxide=44.69 g.  $\text{Ca}(\text{OH})_2$  and moistened with 5 ccm. water. After the mixture has been subjected to considerable pressure and the pressed piece hardened for about two hours by flowing steam superheated to approximately 170° C., the resulting piece has a weight of 124.73 g. and contains 46.46% Mo=57.95 g. Mo.

*Example 2*

To produce acid calcium molybdate  $\text{CaO}_3\text{MoO}_3$ , 90 g. of commercial molybdic acid containing 64.4% Mo=57.96 g. Mo are mixed with 15.2 g. commercial 98 per cent. calcium hydroxide=14.9 g.  $\text{Ca}(\text{OH})_2$  and moistened with 5 ccm. water. After the mixture has been subjected to considerable pressure the pressed piece is placed for a short time in a container filled with water, whereupon the water is evaporated in a drying apparatus. The dried and hardened pressed piece obtained has a weight of 101.7 g. and contains 56.99% Mo=57.96 g. Mo.

*Example 3*

A pressed piece composed of acid calcium molybdate and silicic acid is obtained by mixing 90 g. molybdic acid containing 64.4% Mo=57.96 g. Mo, 15.2 g. commercial 98 per cent. calcium hydroxide=14.9 g.  $\text{Ca}(\text{OH})_2$  and 22.6 g. quartz sand and making a mixture thereof while adding 5 ccm. water. The moist mixture is pressed in molds by applying considerable pressure. The pressed piece is then hardened by subjecting it for instance for two hours to the action of superheated flowing steam. In this way a pressed piece weighing 124.3 g. and containing 46.63% Mo=57.96 g. Mo is obtained.

The expression "an alkaline-earth molybdate", occurring in the appended claims, is intended to include normal or neutral molybdates as well as acid molybdates or polymolybdates.

The expression "molybdic acid" occurring in the appended claims is intended to include molybdic acid itself as well as molybdenum trioxide,  $\text{MoO}_3$ , the anhydride of molybdic acid.

I claim:

1. Process for producing a hard mass containing an alkaline-earth molybdate which comprises subjecting a slightly moist mixture comprising molybdic acid and an alkaline-earth hydroxide to high pressure to form a compacted mass from said mixture and thereafter subjecting the compacted mass to treatment which causes interaction between molybdic acid and al-

kaline-earth hydroxide with the formation of an alkaline-earth molybdate, which interaction is accompanied by hardening of the compacted mass.

2. Process for producing a hard mass containing an alkaline-earth molybdate which comprises subjecting a slightly moist mixture comprising molybdic acid and an alkaline-earth hydroxide to high pressure to form a compacted mass from said mixture and thereafter contacting said compacted mass with steam to harden it.

3. Process for producing a hard mass containing an alkaline-earth molybdate which comprises subjecting a slightly moist mixture comprising molybdic acid and an alkaline-earth hydroxide to high pressure to form a compacted mass from said mixture and thereafter contacting said compacted mass with steam at a temperature above 100° C.

4. Process for producing a hard mass containing an alkaline-earth molybdate which comprises subjecting a slightly moist mixture comprising molybdic acid and an alkaline-earth hydroxide to high pressure to form a compacted mass from said mixture, wetting said compacted mass with water and thereafter drying the wetted compacted mass.

5. Process for producing a hard mass containing an alkaline-earth molybdate which comprises subjecting a slightly moist mixture comprising molybdic acid and an alkaline-earth hydroxide to high pressure to form a compacted mass from said mixture, soaking said compacted mass with water and thereafter drying the mass.

6. Process for producing a hard mass containing an alkaline-earth molybdate which comprises subjecting a slightly moist mixture comprising molybdic acid, an alkaline-earth hydroxide and silicon dioxide to high pressure to form a compacted mass from said mixture and thereafter subjecting the compacted mass to treatment which causes interaction between molybdic acid and alkaline-earth hydroxide with the formation of an alkaline-earth molybdate, which interaction is accompanied by hardening of the compacted mass, the alkaline-earth oxide and silicon dioxide ratio of said mixture corresponding to such ratio of steel furnace slag.

7. Product produced according to claim 1.

8. Product produced according to claim 6.

9. Process for producing a hard mass containing an alkaline-earth molybdate which comprises subjecting a slightly moist mixture comprising molybdic acid and an alkaline-earth hydroxide to high pressure to form a compacted mass from said mixture and thereafter subjecting the compacted mass to the action of water and heat to harden said compacted mass.

10. Process for producing a hard mass, piece or lump containing an alkaline-earth molybdate which comprises subjecting a slightly moist mixture comprising molybdic acid and an alkaline-earth hydroxide to high pressure to form a compacted mass from said mixture and drying the said compacted mass.

11. Product produced according to claim 10.

12. In the art of producing masses, pieces or lumps containing alkaline-earth molybdate, the step which comprises subjecting a slightly moist mixture comprising molybdic acid and an alkaline-earth hydroxide to great pressure to form a compacted mass from said mixture.